

**1****3,577,349****COMPOSITION FOR DESTROYING HARDENED CEMENTITIOUS MIXTURES**

Robert Glenn Haines, South Charleston, W. Va., assignor to Union Carbide Corporation, New York, N.Y.  
No Drawing. Filed Jan. 31, 1969, Ser. No. 795,709  
Int. Cl. C09d 9/00; C11d 7/05; C23g 5/02  
U.S. Cl. 252—170

8 Claims

**ABSTRACT OF THE DISCLOSURE**

A composition for destroying hardened cementitious mixtures comprising methyl acetoacetate and water. A method for destroying hardened cementitious mixtures utilizing said composition is also covered.

This invention relates to a novel composition for destroying hardened concrete and/or cement mortars, and to a process for the removal of hardened concrete and/or cement mortars from various substrates.

Concrete "builds up" on the baffles and other inside surfaces of concrete ready-mix truck drums because of the inability or failure to remove all of the concrete from the ready-mix truck drums before the concrete begins to "set-up." Since concrete adheres better to concrete than to smooth steel, concrete build-up in the ready-mix truck drums enhances more concrete build-up. Because of the angle of the baffles in conventional concrete ready-mix truck drums, rotation of the drum in one direction mixes the drum contents by continuously forcing the upper portion of the contents towards the back or larger closed end of the drum, whereas rotation of the drum in the opposite direction discharges the contents. Any good attempt at washing a ready-mix truck drum by rotating the drum in the "mixing direction," if done before the concrete sets-up, will clean the backside of the baffles in essentially all of the back, larger closed end of the drum. However, the front side of the baffle, and front, smaller end of the drum can only be cleaned by diligent and timely use of a high pressure water spray. All ready-mix trucks have a high pressure water hose with a spray nozzle for this purpose, but when and how this water is used depends of course, on the individual operators of the truck. Depending on the slump of the concrete being hauled ("low-slump" concrete will form build-up in ready-mix truck drums faster than "high-slump" concrete), a "poor" truck operator will have one cubic yard of concrete build-up occur during a period of from 3 to 6 months. A "good" truck operator, i.e., one who regularly and thoroughly cleans the ready-mix drums, may not have this much build-up in more than 3 years. It must be realized, of course, that this more thorough drum cleaning does require operator time which may well result in an average of one less truck-load per day of concrete delivered. Once there is concrete build-up in the truck drum, there are various conventional ways in which

**2**

it can be removed. Most ready-mix concrete firms use coarse aggregate and water with drum rotation and/or air hammers to remove the concrete build-up from their truck drums. Other firms, use "shaped" dynamite charges to destroy the concrete build-up. Either of these two latter methods, however, can cause considerable damage to the drums not to mention the danger involved with these methods. There are other problem areas in the art wherein concrete build-up presents problems. For example, concrete build-up is very detrimental to construction equipment, such as to precast forms, form clamps, mortar boxes, laboratory forms and other tools. The use of dynamite charges and other physical means for removing this concrete build-up in construction equipment is obviously undesirable. More recently, the art has relied heavily on chemical compounds and/or compositions which can be employed as concrete dissolvers. Various organic and inorganic compounds have been found to be effective for this purpose. The inorganic compounds which are useful as concrete dissolvers generally include inorganic acids such as hydrochloric, phosphoric, hypochlorous and carbonic acid. Salts of these acids and alkalies such as sodium-hydroxide, sodium bicarbonate and ammonium-sulfate are also effective. The organic chemicals which have been found to be effective as concrete dissolvers generally include organic acids such as oxalic, acetic, lactic, citric, tannic and humic acid as well as combinations of these acids and other organic compounds such as anhydrides or ethers of the above, the most widely used being hydrochloric or muriatic acid. Use of acids whether organic or inorganic for dissolving and/or destroying cementitious mixtures of course, present safety hazards whereas other known compounds although somewhat effective for destroying concrete, unfortunately, also destroy or reduce the desirable properties of cementitious mixtures even when present in minute, residual concentrations. It should be remembered that although a chemical compound may be effective for destroying concrete, inadvertent, residual concentrations of it should nevertheless be compatible with new batches of concrete or cementitious mixtures since there generally remain on the surface from which the concrete was removed, residual amounts of the chemical compound or dissolver. Thus there is still a need in the art for a concrete destroyer which is easy to apply, safe to use, and which possess properties which do not harmfully affect the properties of new cementitious mixtures such as compressive strength, setting time and durability.

It is therefore an object of the present invention to provide a novel composition for destroying hardened cementitious mixtures such as concrete and/or cement mortars.

Another object is to provide a process for the removal of hardened concrete and/or cement mortars from various substrates. Another object is to provide a novel composition for destroying hardened concrete inadvertently residual traces of which does not adversely affect the properties of newly mixed concrete. These and other

objects will be apparent from the following description of the invention.

As employed herein, the term cementitious mixtures is meant to include concrete, cement mortars, cinder blocks, masonry mortars, concrete lintels, concrete pipe, cement-asbestos pipe, prestressed concrete and the like.

In an effort to provide a hardened cementitious destroyer such as a hardened concrete or mortar destroyer, which is easy to apply, safe to use, and residual traces of which does not affect the properties of new batches of freshly prepared cementitious mixtures I tried various compounds such as: ethylacetoacetate, alpha-chloroethylacetoacetate, ethyl levulinate, methyl levulinate, methyl pyruvate, methyl propionate and methyl chloroacetate. None of these compounds however, were found to be effective in destroying hardened cementitious mixtures with the exception of ethylacetoacetate which was found to possess a degree of effectiveness on very young concrete, i.e., 8 hour old concrete. However, ethylacetoacetate had little or no effect on older concrete, i.e., 24 hour concrete.

During the course of this experimentation, I tried methyl acetoacetate, a compound closely chemically related to the above compounds, and found surprisingly, and contrary to normal expectations that the methyl acetoacetate was extremely effective in destroying hardened concrete and this destructive ability was maintained in treating young as well as old concrete. Advantageously, it was found that in mixing new batches of concrete in equipment previously treated with methyl acetoacetate, that the new batches suffered little or no detrimental effects, and in fact there was actually an increase in the compressive strength of the new concrete which is attributed to the presence of the methyl acetoacetate or more correctly, to the reaction product of methyl acetoacetate and cement.

Broadly contemplated, the present invention provides a composition for destroying hardened cementitious mixtures which comprises methyl acetoacetate and water. More specifically, the composition for destroying hardened cementitious mixtures comprises from about 60% to 99% by weight methyl acetoacetate, and from about 1 to 40% water. Optionally, though desirably, there can be included in the composition a penetrating aid which has been found to increase the aggressiveness of the methyl acetoacetate water solution to the hardened cementitious mixture.

The methyl acetoacetate solution can be applied to the surface of the hardened cementitious mixture to be destroyed in any convenient manner known in the art. When the hardened cementitious mixture is present on exposed accessible surfaces such as on tools, mortar boxes, clamps, precast forms, and the like, the methyl acetoacetate water solution can be applied directly to the surface such as by pouring, spraying, dipping and the like. To reach inaccessible enclosed areas, such as the inner area of a drum of a ready-mix truck, the methyl acetoacetate solution is added to the enclosed area and the system agitated sufficiently to permit the solution to come in contact with any hardened cementitious mixture adhering to the drum including the baffles of the drum.

The methyl acetoacetate-water solution apparently destroys the hardened cementitious mixture by reacting with the cement phase of the mixture. Application of the methyl acetoacetate to the hardened cementitious mixture produces a detectable heat of reaction and ultimately there results a low-density "powder-like" solid together with a yellow-orange liquid product. As a result of the reaction, the chemical composition of the cement phase is changed (a portion of the cement phase is actually solubilized) and the hardened cementitious mixture is destroyed.

The amount of methyl acetoacetate employed in the methyl acetoacetate-water solution can be varied over

a relatively wide range and depends in part, upon the age of the hardened cementitious mixture to be destroyed as well as the length of time available for destruction. Generally, in treating "young" hardened cementitious mixtures there can be employed as little as 25% methyl acetoacetate by weight, although higher concentrations such as 50% and 85% methyl acetoacetate by weight results in more destructive power in appreciably shorter periods of time. Merely as illustrative an 85 weight percent solution of methyl acetoacetate destroyed a 12 hour old concrete specimen (prepared with limestone coarse aggregate) in about 3 minutes, whereas 50 and 25 weight percent solution of methyl acetoacetate required 5 minutes and 40 minutes, respectively, to dissolve similar concrete specimens. Relatively similar results are achieved in treating older concrete, for example, in treating concrete which was about 17 hours old, with 85, 50 and 25 weight percent solutions of methyl acetoacetate, the time required to destroy the concrete was about 65, 80 and 300 minutes respectively. Thus, although some water is necessary for achieving maximum effectiveness in destroying concrete, too much water i.e., substantially more than 15 weight percent water merely dilutes and so decreases the rate of concrete dissolution. Excellent results are obtained when the methyl acetoacetate in the methyl acetoacetate-water solution is in the range of about 80 to 90% preferably about 85% by weight of the solution.

Optionally, and desirably, there can be included in the composition, a penetrating aid, which as its name indicates, serves to facilitate contact of the destroyer solution with the hardened cementitious mixture. A wide variety of penetrating aids can be employed for this purpose such as a detergent type penetrating aid of the anionic, non-ionic or cationic type.

Illustrative of the anionic type penetrating aids are the alkyl sulfates or ethoxy sulfates of secondary alcohols such as the sodium sulfate of tetradecanol; sodium sulfate of 2-methyl - 7 - ethyl undecanol-4 (Tergitol 4); sodium sulfate of 3,9 - diethyl tridecanol-6 (Tergitol 6) and the sodium ethoxysulfate of C<sub>11</sub> to C<sub>15</sub> linear, secondary alcohols (Tergitol 15-S-3S).

Illustrative of the non-ionic type penetrating aids are the ethoxylates of branched secondary alcohols such as the ethoxylate of 2,6,8-trimethyl - 4 - nonanol (Tergitol 15-S-3) and the 9 mol ethoxylate of C<sub>11</sub> to C<sub>15</sub> linear, secondary alcohols, Tergitol 15-S-9).

Illustrative of a cationic type penetrating aid is 1-hydroxyethyl-2-heptadecenyl glyoxalidine.

The above penetrating aids may be obtained from Union Carbide Corporation under the trademark Tergitol.

The penetrating aid can be added to the composition in an amount of up to about 5% by weight preferably about 0.5% by weight based on the weight of the composition.

The methyl acetoacetate to hardened cementitious mixture weight ratio can also be varied over a relatively wide range as from about 0.01 to 2 parts by weight methyl acetoacetate to 1 part by weight hardened cementitious mixture preferably 0.1 to 1 part by weight methyl acetoacetate to 1 part by weight hardened cementitious mixture.

The following examples will illustrate the present invention.

#### EXAMPLES 1 THROUGH 30

In these examples, the effect of concrete age and methyl acetoacetate solution concentration on destruction time is illustrated. "Static tests" were performed on the specimen, i.e., weighed specimens were immersed in a vessel containing the methyl acetoacetate solution and the specimens were checked periodically for weight loss. In Examples 1 to 3, the concrete specimens were broken concrete test cylinders and in Examples 4 to 30, the concrete specimens were 2" x 2" x 2" blocks. The concrete age, concentrations, course aggregate used, and results are summarized for convenience in Table I below.

TABLE I.—“STATIC” TESTS WITH METHYL ACETOACETATE/WATER SOLUTIONS THE EFFECTS OF CONCRETE AGE AND METHYL ACETOACETATE SOLUTION CONCENTRATION ON DESTRUCTION TIME

| Example | Concrete age | Methyl acetoacetate conc. in solution, wt. percent | Methyl acetoacetate to concrete wt. ratio | Time required to destroy concrete        | Coarse aggregate used in concrete |
|---------|--------------|----------------------------------------------------|-------------------------------------------|------------------------------------------|-----------------------------------|
| 1       | 2 days       | 85                                                 | 1.0                                       | 1.0 hr.                                  | Limestone.                        |
| 2       | 90 days      | 85                                                 | 1.0                                       | 1.7 hrs.                                 | Do.                               |
| 3       | do           | 85                                                 | 1.0                                       | 3.0 hrs.                                 | Do.                               |
| 4       | 4 hours      | 85                                                 | 1.0                                       | 2 mins.                                  | Do.                               |
| 5       | do           | 50                                                 | 0.5                                       | 4 mins.                                  | Do.                               |
| 6       | do           | 25                                                 | 0.25                                      | 15 mins.                                 | Do.                               |
| 7       | do           | 85                                                 | 1.0                                       | 1 min.                                   | Ohio river gravel.                |
| 8       | do           | 50                                                 | 0.5                                       | 2 mins.                                  | Do.                               |
| 9       | do           | 25                                                 | 0.25                                      | 20 mins.                                 | Do.                               |
| 10      | 7 hours      | 85                                                 | 1.0                                       | 6 mins.                                  | Limestone.                        |
| 11      | do           | 50                                                 | 0.5                                       | 12 mins.                                 | Do.                               |
| 12      | do           | 25                                                 | 0.25                                      | 50 mins.                                 | Do.                               |
| 13      | do           | 85                                                 | 1.0                                       | 1 min.                                   | Ohio river gravel.                |
| 14      | do           | 50                                                 | 0.5                                       | 2 mins.                                  | Do.                               |
| 15      | do           | 25                                                 | 0.25                                      | 25 mins.                                 | Do.                               |
| 16      | 9 hours      | 85                                                 | 1.0                                       | 37% dissolved in 31 hrs.; specimen soft. | Do.                               |
| 17      | do           | 50                                                 | 0.5                                       | 17% dissolved in 31 hrs.; specimen soft. | Do.                               |
| 18      | do           | 25                                                 | 0.25                                      | 7% dissolved in 31 hrs.; specimen solid. | Do.                               |
| 19      | 12 hours     | 85                                                 | 1.0                                       | 3 mins.                                  | Limestone.                        |
| 20      | do           | 50                                                 | 0.5                                       | 5 mins.                                  | Do.                               |
| 21      | do           | 25                                                 | 0.25                                      | 40 mins.                                 | Do.                               |
| 22      | do           | 85                                                 | 1.0                                       | 85% dissolved in 9 hours.                | Ohio river gravel.                |
| 23      | do           | 50                                                 | 0.5                                       | 29% dissolved in 9 hours.                | Do.                               |
| 24      | do           | 80                                                 | 0.25                                      | 6% dissolved in 9 hours.                 | Do.                               |
| 25      | 14.5 hours   | 80                                                 | 1.0                                       | 15 mins.                                 | Limestone.                        |
| 26      | do           | 50                                                 | 0.5                                       | 81% dissolved in 129 hours.              | Do.                               |
| 27      | do           | 25                                                 | 0.25                                      | 14% dissolved in 129 hours.              | Do.                               |
| 28      | 17 hours     | 80                                                 | 1.0                                       | 38% dissolved in 71 hours.               | Do.                               |
| 29      | do           | 50                                                 | 0.5                                       | 18% dissolved in 71 hours.               | Do.                               |
| 30      | do           | 25                                                 | 0.25                                      | 10% dissolved in 71 hours.               | Do.                               |

TABLE II.—“ROLLING” TESTS WITH METHYL ACETOACETATE/WATER SOLUTIONS IN BAFFLED, FIVE-GALLON CONTAINERS

30 The effect of concrete age and methyl acetoacetate solution concentration on destruction time

| Example | Concrete age | Methyl acetoacetate conc. in solution, wt. percent | Methyl acetoacetate to concrete, wt. ratio | Time required to destroy concrete, minutes |
|---------|--------------|----------------------------------------------------|--------------------------------------------|--------------------------------------------|
| 31      | 7 hours      | 85                                                 | 1.0                                        | 15                                         |
| 32      | do           | 70                                                 | 0.5                                        | 20                                         |
| 33      | do           | 25                                                 | 0.25                                       | 45                                         |
| 34      | do           | 25                                                 | 0.125                                      | 50                                         |
| 35      | 10.5 hours   | 50                                                 | 0.5                                        | 20                                         |
| 36      | do           | 25                                                 | 0.25                                       | 60                                         |
| 37      | do           | 25                                                 | 0.125                                      | 120                                        |
| 38      | do           | 25                                                 | 0.063 <sup>1</sup>                         | 120                                        |
| 39      | 17 hours     | 85                                                 | 1.0                                        | 65                                         |
| 40      | do           | 50                                                 | 0.5                                        | 80                                         |
| 41      | 18.5 hours   | 25                                                 | 0.25                                       | 300                                        |
| 42      | do           | 25                                                 | 0.125                                      | 300                                        |
| 43      | 20 hours     | 25                                                 | 0.25                                       | 300                                        |
| 44      | 22 hours     | 85                                                 | 1.0                                        | 75                                         |
| 45      | 24 hours     | 85                                                 | 1.0                                        | 180                                        |
| 46      | do           | 50                                                 | 0.5                                        | 180                                        |
| 47      | do           | 50                                                 | 0.5                                        | 100                                        |
| 48      | do           | 25                                                 | 0.25                                       | 720                                        |

<sup>1</sup> Apparently not enough methyl acetoacetate present.

## EXAMPLES 49 THROUGH 52

50 These examples demonstrate the effect of a penetrating aid for the methyl acetoacetate solution in destroying concrete. In Example 50 the penetrating aid employed was Tergitol 7, an anionic detergent (sodium heptadecyl sulfate) available from Union Carbide Corporation. In Example 51, the penetrating aid employed was Tergitol TMN a non-ionic detergent (trimethyl nonanol polyethylene glycol ether) available from Union Carbide Corporation and in Example 52, the penetrating aid was Teritol amine 220, a cationic detergent (hydroxylalkyl alkenyl glyoxalidine). For convenience the characteristics and results of the tests are indicated in Table III.

55 60

TABLE III.—“STATIC” TESTS: THE EFFECTS OF VARIOUS TYPES OF DETERGENTS AS PENETRATING AIDS FOR METHYL ACETOACETATE IN DESTROYING CONCRETE

Concrete specimens: 2" x 2" x 2" concrete cubes. Ohio river gravel coarse aggregate  
Weight ratio: Water-chemical-concrete=15-100-100  
Concrete age=8 hours

| Ex. | “Dissolver” solution                                                    | Contact time                 |                                                              |                              |
|-----|-------------------------------------------------------------------------|------------------------------|--------------------------------------------------------------|------------------------------|
|     |                                                                         | 1 hour                       | 23 hours                                                     | 27 hours                     |
| 49  | Methyl acetoacetate                                                     | Cube 81% of original weight. | Cube 57% of original weight. Reaction product a heavy paste. | Cube 54% of original weight. |
| 50  | Methyl acetoacetate plus 0.5 wt. percent TERGITOL 7 (anionic).          | Cube 75% of original weight. | Cube 17% of original weight.                                 | Cube disintegrated.          |
| 51  | Methyl acetoacetate plus 0.5 wt. percent TERGITOL TMN (non-ionic).      | Cube 70% of original weight. | Cube 16% of original weight.                                 | Cube 13% of original weight. |
| 52  | Methyl acetoacetate plus 0.5 wt. percent TERGITOL AMINE 220 (cationic). | Cube 84% of original weight. | Cube 42% of original weight.                                 | Cube 41% of original weight. |

7  
EXAMPLE 53

The example demonstrates the effectiveness of methyl acetoacetate and compares its effectiveness with inhibited hydrochloric acid (38 wt. percent). The hydrochloric acid was inhibited with alkyl pyridine HB. The test characteristics and results are indicated in Table IV.

## 8

85% by weight methyl acetoacetate, about 14.5% water by weight and about 0.5% penetrating aid.

3. A composition according to claim 2 wherein said hardened cementitious mixture is concrete.

4. A process for destroying hardened cementitious mixtures which comprises contacting said hardened cementitious mixture, with a composition consisting essentially of

TABLE IV

| Chemical                                          | Weight ratio,<br>Water-Chemical-Specimens | pH of<br>mixtures | Contact<br>time,<br>hours              | Remarks                                                                                                                                                                                                                      |
|---------------------------------------------------|-------------------------------------------|-------------------|----------------------------------------|------------------------------------------------------------------------------------------------------------------------------------------------------------------------------------------------------------------------------|
| Methyl acetoacetate.....                          | 25      148                               | 148               | 4.0<br>5.0<br>5.5<br>6.4<br>6.4<br>1.0 | 0 Small pieces falling from specimen.<br>1 Solution amber colored.<br>2 Specimen 90% of original weight.<br>5 Specimen 76% of original weight.<br>7 Specimen 57% of original weight.<br>24 Noting left but paste and stones. |
| Inhibited hydrochloric acid (36 wt. percent)..... | 2,210<br>(10% HCl)                        | 790               | 300                                    | 1 Specimen 95% of original weight.<br>18 Specimen 86% of original weight.<br>21 Specimen 81% of original weight.                                                                                                             |

As will be evident and from the above examples a 20 water solution of methyl acetoacetate is extremely effective as a concrete destroyer and the most effective concentration is an 85/15 weight percent methyl acetoacetate water solution. The effectiveness is even more pronounced when a penetrating aid is added to the solution. Although, a water solution of methyl acetoacetate is somewhat corrosive, corrosion tests on mild steel indicated that metal lost due to corrosion from the use of methyl acetoacetate to dissolve the concrete build-up that occurs in ready-mix concrete truck drums is not a significant factor in the useful life of the drums. This is because the reaction product of methyl acetoacetate, water and concrete is less corrosive to mild steel than water solutions of methyl acetoacetate. Moreover, no permanent detrimental effects were obtained in 24 hour immersion (immersion in eighty-five weight percent methyl acetoacetate-water solutions) tests on neoprene, black rubber, black gum rubber, rubber latex, polyethylene or tygon tubing. Thus, the methyl acetoacetate solution can be employed with tools or equipment fabricated from these materials.

What is claimed is:

1. A composition for destroying hardened cementitious mixtures consisting of methyl acetoacetate in an amount of about 60-99% by weight, water in an amount of about 1-40% by weight and a penetrating aid selected from the group consisting of anionic, nonionic or cationic detergents in an amount of about 0.5-5% by weight.

2. A composition according to claim 1 containing about

20 methyl acetoacetate in an amount of about 60-99% by weight and water in an amount of about 1-40% by weight for a time sufficient to destroy said hardened cementitious mixture.

25 5. A process according to claim 4 wherein said composition is employed in an amount of about 0.1 to 1% by weight based on the weight of the hardened cementitious mixture.

30 6. A process according to claim 4 wherein said composition also includes a penetrating aid selected from the group consisting of anionic, nonionic or cationic detergents.

35 7. A process according to claim 6 wherein said methyl acetoacetate, said water and said penetrating aid are employed in an amount of about 85%, 14.5% and 0.5% by weight respectively.

8. A process according to claim 7 wherein said hardened cementitious mixture is concrete.

## References Cited

40 Rose: The Condensed Chem. Dict. 6th Ed., Reinhold Publ. Co., 1961, p. 729.

LEON D. ROSDOL, Primary Examiner

45 W. E. SCHULZ, Assistant Examiner

U.S. Cl. X.R.

106-311; 134-2, 23; 252-89